

Feb. 9, 1971

B. D. ALLAN ET AL

3,562,035

DESENSITIZATION OF DIFLUOROAMINO-SUBSTITUTED PROPELLANT  
COMPOUNDS USING DINITROGEN TETRAOXIDE

Filed Sept. 10, 1962

SENSITIVITY V. MOLAR RATIO



Barry D. Allan  
Edgar F. Croomes  
Walter W. Wharton,  
INVENTORS.

BY *S. J. Rotondi*  
*A. L. Dusant*  
*Jack W. Voigt*

## 1

3,562,035

## DESENSITIZATION OF DIFLUOROAMINO-SUBSTITUTED PROPELLANT COMPOUNDS USING DINITROGEN TETRAOXIDE

Barry D. Allan, Edgar F. Croomes, and Walter W. Wharton, Huntsville, Ala., assignors to the United States of America as represented by the Secretary of the Army  
Filed Sept. 10, 1962, Ser. No. 222,738  
Int. Cl. C06b 19/06

U.S. CL. 149—74

## 3 Claims

The invention described herein may be manufactured and used by or for the Government for governmental purposes without the payment of any royalty thereon.

This invention relates to the stabilization of rocket fuels employed in liquid monopropellant and liquid bipropellant systems. More particularly, this invention is concerned with the stabilization of difluoroamino-substituted compounds employed as fuels and/or oxidizers in rocket propulsion systems.

Recent developments in rocket fuels have been directed towards the preparation of propellants which will afford higher specific impulses than those propellants utilized heretofore. Theoretical calculations indicate that propellants based on a carbon-hydrogen-oxygen-nitrogen-fluorine system will exceed appreciably the specific impulse of propellants based only on a carbon-hydrogen-oxygen-nitrogen system. Therefore, a whole new class of propellants based on difluoroamino-substituted compounds has evolved.

One problem immediately became apparent in work with difluoroamino-substituted fuels. These fuels, because of the sensitivity of difluoroamino groups, had a tendency to detonate at low-shock sensitivity values. This sensitivity requires the use of special handling techniques to prevent premature detonation of the fuel.

For application to rockets, especially military rockets, special handling requirements for a fuel are a distinct disadvantage and may even eliminate the fuel or rockets employing the fuel from consideration. To render these new fuels acceptable to military needs and thereby afford military rockets the advantages of the higher specific impulse of these fuels required a means of reducing their shock sensitivity.

It has now been determined that these difluoroamino-substituted fuels may be effectively desensitized without adversely affecting the propulsion performance thereof by adding trace amounts of dinitrogen tetraoxide to the fuel.

In view of the above, it is the object of the invention to set forth an effective means of desensitizing difluoroamino-substituted compounds by adding to said compounds dinitrogen tetraoxide thereby preventing premature detonation due to shock.

The manner in which this and other objects may be achieved will become apparent from the following discussion.

The graph illustrates the amount of desensitization achieved when a typical difluoroamino-substituted compound is treated with dinitrogen tetraoxide.

The liquid difluoroamino-substituted compounds desensitized thus far appear to be completely miscible with the dinitrogen tetraoxide. Therefore, all that is required to achieve the desensitization of these compounds to shock is a simple mixing of the two components. The molar ratio of the difluoroamino-substituted compound to the dinitrogen tetraoxide should be at least 1.0:0.004. There is little if any advantage in employing a molar ratio in excess of one mole of dinitrogen tetraoxide to each mole of difluoroamino-derivative.

## 2

For ordinary use as rocket propellant components, the difluoroamino-derivatives are rendered sufficiently insensitive to shock when a molar ratio of difluoroamino-derivative to dinitrogen tetraoxide of 1.0:0.004 to 1.0:0.3 is employed. However, because the dinitrogen tetraoxide can function as an oxidizer for the difluoroamino-derivatives, the use of more than trace amounts of dinitrogen tetraoxide with the difluoroamino-derivatives is completely acceptable.

10 In mixing the dinitrogen tetraoxide with the difluoroamino derivative to be desensitized, the relatively low boiling point (B.P. 21.3° C.) of dinitrogen tetraoxide should be considered. Working with temperatures below this point prevents undue loss of the desensitizing material during mixing and storage. Nevertheless, since even trace amounts of the desensitizer function successfully, low temperature requirements are not necessary but merely advantageous.

15 The manner in which desensitization is achieved is not completely understood. However, it is believed that the decomposition of the difluoroamino derivatives, which accompany the shock and lead to detonation, is terminated by a reaction between the decomposition product of the difluoroamino derivative and the nitrogen dioxide which is present in the dinitrogen tetraoxide. This reaction halts the decomposition before detonation occurs. The nature of the reaction is unknown but apparently the available electron in the nitrogen dioxide readily reacts with the decomposition product. Nitrogen dioxide is the product 20 of the dissociation of dinitrogen tetraoxide in solution (see Moeller, Inorganic Chemistry, published by John Wiley and Sons, Inc., New York, 1952).

25 There is some evidence that the desensitization is achieved according to the postulated method. If trace amounts of 1,1 - diphenyl - 2(2',4',6' - trinitrophenyl)-hydrazine is added in trace amounts to the liquid difluoroamino-substituted compounds, desensitization is also achieved. Like the nitrogen dioxide, this compound also furnishes an available electron which apparently 30 enters into some type of reaction with the decomposition products resulting from shock. Thus, it would appear that any substance which is capable of producing free-radicals would function as desensitizers. However nitrogen tetraoxide is the preferred desensitizer of the invention.

35 It is to be understood that the above discussion is merely an attempt to explain the desensitization process and is in no way to be interpreted as a limitation of the invention. Regardless of the mechanism by which desensitization 40 is accomplished, the method of the invention for desensitizing difluoroamino - substituted compounds achieves the desired result, the mechanism being immaterial to the successful employment of the method of desensitization.

45 Among the difluoroamino-substituted compounds which have been desensitized by the dinitrogen tetraoxide are the tetrafluorohydrazine adducts of ethylenically unsaturated compounds such as 2-methyl-propene, 4-methyl-pentene-1, and methyl methacrylate. Generally speaking, these 50 adducts are prepared by reacting the unsaturated compound with tetrafluorohydrazine at sub-atmospheric or super-atmospheric pressure. The operable temperature range for the process is from 40° C. to 150° C. Since one mole of tetrafluorohydrazine is required for each double 55 bond in the unsaturated compound, at least one mole of tetrafluorohydrazine is required for every mole of mono-ethylenically unsaturated reactant. However, an excess of up to five moles of the tetrafluorohydrazine will increase the yields and/or shorten the reaction time.

60 A preferred class of tetrafluorohydrazine adducts suit-

able as propellant fuels which can be desensitized according to the process of the invention are those of the formula



wherein R, R', R'', and R''' are each members selected from the group consisting of hydrogen and branched and straight chain lower alkyl groups of up to four carbon atoms. The total carbon content of R, R', R'', and R''' should not exceed six, however.

The following examples are illustrative of the preparation of these difluoroamino adducts.

#### EXAMPLE I

##### 1,2-bis (difluoroamino) propane

To a 500 cc. evacuated Pyrex bulb equipped with stopcock and condensing arm was added in vacuo  $6.4 \times 10^{-3}$  mole crude tetrafluorohydrazine and  $6.1 \times 10^{-3}$  mole propylene. The bulb, equipped with a capillary monometer, was placed in an oil bath and maintained at 100° C. to 110° C. for eight hours. The pressure decreased from 518 mm. (106° C.) to 316 mm. (106° C.) during this period. The bulb was then removed from the bath and the condensing arm immersed in a bath at -196° C. A slight pressure of noncondensable gas was pumped from the bulb, the material remaining in the bulb being subsequently warmed to room temperature and transferred into the vacuum system. Some non-volatile material remained in the bulb. The material which transferred to the vacuum system was fractionated through traps. The fraction collected at -96° C. was a colorless liquid with a reproducible vapor pressure of 21 mm. at 0° C. A molecular weight determination on an aliquot of the fraction by the gas density method gave value of 146.9;  $\text{C}_3\text{H}_4\text{N}_2\text{F}_4$  requires 146.1. The fraction weighed 0.45 gram which corresponds to a 60% yield based on tetrafluorohydrazine consumption.

Calculated for  $\text{C}_3\text{H}_4\text{N}_2\text{F}_4$  (percent): C, 24.66; H, 4.14; N, 19.18; F, 52.02. Found (percent): C, 24.72; H, 4.74; N, 18.05; F, 49.9.

#### EXAMPLE II

##### 1,2-bis (difluoroamino) propane

A 1.5:1 molar ratio of tetrafluorohydrazine to propylene was heated at 110° C. in a 500 cc. stainless steel bomb for two and one-half hours. The pressure decreased from 72 p.s.i. (25° C.) to 21 p.s.i. (25° C.) during this period. The product was distilled under an atmosphere of nitrogen yielding almost 6 grams of 1,2-bis (difluoroamino) propane having a boiling point of 83-84° C. at a pressure of 760 mm. This corresponds to approximately a 90% yield based on the propylene employed.

#### EXAMPLE III

##### 1,2-bis (difluoroamino)-2-methyl-propane

Following the procedure of Example I, a mixture of tetrafluorohydrazine and isobutylene, in a molar ratio of tetrafluorohydrazine to isobutylene of 1.27:1, was heated at 110° C. for six hours. During the course of the reaction the pressure of the mixture dropped from 496.2 mm. (28.1° C.) to 95 mm. (25.2° C.). After heating, the reaction mass was cooled to room temperature. The desired product was again recovered by fractionation yielding 3.6 g. (86% yield) of a liquid having a boiling point of 99.5-100° C. The product gave vapor pressure of 12.1 mm. at 0.0° C., 26.1 mm. at 15.0° C., and 49.3 mm. at 27.8° C. Quantitative hydrolysis of 61.06 mg. in 35.99 ml. of 0.1110 N sodium hydroxide-10 ml. ethanol solution for twenty-one hours gave an equivalent weight of 40.14; calculated equivalent weight 40.0.

Calculated for  $\text{C}_4\text{H}_6\text{N}_2\text{F}_4$  (percent): F, 47.5. Found (percent): F, 47.2.

By substituting methyl methacrylate, 4-methyl-pentene-

1, butene-1, and other ethylenically unsaturated compounds for the propylene and isobutylene of Examples I-III, the tetrafluorohydrazine adducts of these compounds can be synthesized.

The degree of desensitization achieved through the use of dinitrogen tetraoxide was determined through the use of the Olin Mathieson drop weight tester. This test has been approved by the Joint-Army-Navy-Air Force Panel on Liquid Propellant Test Methods. Essentially, this tester is used to determine what shock will cause the non-desensitized material to detonate fifty percent of the time. The shock is achieved by dropping various weights measured distances to subject the material being tested to the impact thus produced. Then the material is desensitized and subjected to the test again. The increase in the amount of weight and/or distance the weight is dropped to produce fifty percent detonations when compared to the weights and distances for the non-desensitized material provides a means of evaluating the degree of desensitization accomplished.

The effectiveness of dinitrogen tetraoxide as a desensitizer is illustrated in the graph which shows the amount of desensitization achieved when various molar ratios of dinitrogen tetraoxide are added to 1,2-bis (difluoroamino)-2-methyl-propane, an especially suitable rocket fuel within the preferred class of fuels previously mentioned hereinabove. Generally, when the  $E_{50}$  value of the test is greater than 120, the material being tested is considered insensitive to shock. This  $E_{50}$  value is expressed in kg.-cm. and is the product obtained by multiplying the weight which is dropped, measured in kilograms, times the distance the weight is dropped, measured in centimeters.

The  $E_{50}$  value for the pure 1,2-bis (difluoroamino)-2-methyl-propane is 6.9 kg.-cm. Since the graph does not clearly denote the amount of desensitization achieved when dinitrogen tetraoxide is employed in trace amounts, some  $E_{50}$  values for those trace amounts are given hereinafter. When the molar ratio of 1,2-bis (difluoroamino)-2-methyl-propane to dinitrogen tetraoxide is 1.0:0.004, the  $E_{50}$  value is 41 kg.-cm.; when 1.0:0.03, the  $E_{50}$  value is 46 kg.-cm.; when 1.0:0.56, the  $E_{50}$  value is 103 kg.-cm.

The amount of desensitization achieved with other homologous members of the previously identified preferred class of tetrafluorohydrazine adducts is closely analogous to that shown in the graph for the isobutylene adduct.

Another distinct advantage of the desensitizing agent of the invention is its compatibility with the difluoroamino-substituted fuels. Compatibility studies show that the reactivity of dinitrogen tetraoxide towards the difluoroamino derivatives is dependent upon the concentration of dinitrogen tetraoxide and the temperature. When a molar ratio of the tetrafluorohydrazine adduct of isobutylene to dinitrogen tetraoxide of 1.0:1.5 was subjected to prolonged heating at 100° C., reaction or decomposition definitely occurred. This problem is also encountered with other difluoroamino derivatives if the concentration of dinitrogen tetraoxide is relatively high (for example, one-half mole to one and one-half moles of dinitrogen tetraoxide to difluoroamino derivative) and the temperature is maintained at 70° C. or higher. However, prolonged heating of the tetrafluorohydrazine adducts of the alkenes at temperatures of 50° C. to 60° C. does not give evidence of reaction or decomposition even at higher levels of dinitrogen tetraoxide concentration. Illustrative of this is the absence of any reaction or decomposition when a molar ratio of the tetrafluorohydrazine adduct of isobutylene to dinitrogen tetraoxide of 1.0:1.5 is maintained at a temperature of 50° C. to 60° C. for several days. When only trace amounts of dinitrogen tetraoxide are present there is no problem of decomposition or reaction below 100° C.

The difluoroamino derivatives desensitized according to the method of this invention can be employed in the bipropellant rocket motors. Suitable oxidizers for the fuels

include red fuming nitric acid and dinitrogen tetraoxide. The fuel and oxidizer can be injected into the combustion chamber and ignited in a conventional manner as, for example, by first igniting a butane and air mixture. However, the operation of rocket engines is well within the skill of the art and no detailed discussion is necessary herein.

From the foregoing discussion it should be readily apparent to those skilled in the art that the shock desensitization method of the invention is broadly applicable to desensitizing any difluoroamino-substituted compound, particularly liquid compounds. However, solid difluoroamino-substituted compounds which are soluble in liquid dinitrogen tetraoxide or are soluble in a liquid which is also a solvent for dinitrogen tetraoxide can be desensitized according to the method described herein.

Moreover, while the major use for difluoroamino-substituted compounds at the present time is as rocket fuels, this method of desensitization will find further application when the uses for difluoroamino derivatives spread to other areas.

While the invention has been described by reference to specific details thereof, it is not intended that the invention be construed as limited to these details except insofar as they appear in the appended claims.

We claim:

1. The method of desensitizing to shock a difluoroamino-substituted compound of the formula



wherein R, R', R'', and R''' are each members selected from the group consisting of hydrogen and branched and straight chain lower alkyl groups of up to four carbon

atoms, the total number of carbon atoms present in R, R', R'', R''' not to exceed six; said method comprising admixing with said compound dinitrogen tetroxide in the molar ratio of difluoroamino-substituted compound to dinitrogen tetroxide of 1.0:0.004 to 1.0:0.3.

5 2. The method of desensitizing to shock 1,2-bis(difluoroamino)-2-methylpropane by admixing therewith dinitrogen tetroxide in the molar ratio of 1,2-bis(difluoroamino)-2-methyl-propane to dinitrogen tetroxide of 1.0:0.004 to 1.0:0.3.

10 3. The method of desensitizing to shock the tetrafluorohydrazine adduct of a mono-ethylenically unsaturated compound, said adduct being the addition reaction product of one mole of tetrafluorohydrazine with one mole of 15 said compound and being characterized by the presence of the group



20

said method comprising admixing dinitrogen tetroxide with said adduct, the amount of adduct to dinitrogen tetroxide being in a molar ratio of 1.0:0.004 to 1.0:0.3.

25

#### References Cited

#### UNITED STATES PATENTS

3,310,444 3/1967 Gould \_\_\_\_\_ 149—74  
30 3,345,821 10/1967 Magee \_\_\_\_\_ 60—217X

BENJAMIN R. PADGETT, Primary Examiner

U.S. Cl. X.R.

35 60—214; 149—1, 109; 260—583